

## UNITED STATES PATENT OFFICE.

OTTO PATTERMANN, OF KĽADNO, CZECHOSLOVAKIA, ASSIGNOR TO POLDIHÜTTE, OF PALACKEHO TRIDA, PRAHA-VINOHRADY, CZECHOSLOVAKIA, A JOINT-STOCK COMPANY.

## STEEL.

No Drawing. Application filed January 29, 1926, Serial No. 84,754, and in Germany January 8, 1925.

Tools and constructional parts which must be of high strength and tenacity and must retain these properties at high working temperatures, such as dies, swages, valves for high temperature explosion-motors, valve-springs for service with superheated steam; parts of fire arms and the like, are frequently produced from chromium-tungsten steel. In so far as this steel is considerably alloyed, it is not tenacious enough for many purposes and, moreover, a complicated heat treatment of objects manufactured therefrom is necessary. Less considerably alloyed chromium-tungsten-steel, while easier to treat, loses its strength and becomes soft at high working temperatures.

According to the invention, a steel suitable for objects employed at high temperatures and answering all requirements in a most satisfactory manner is produced by the addition of nickel to a chromium-tungsten steel containing at least 3% tungsten. The new steel is hard and tenacious, retains its strength at high temperatures and, moreover, presents no difficulties in the heat treatment during the manufacture of the objects.

The following composition is given as an example of the new steel:

|          | Per cent. |
|----------|-----------|
| Carbon   | 0.3       |
| Chromium | 3.0       |
| Tungsten | 10.0      |
| Nickel   | 3.0       |

The following steel was employed heretofore as the best steel for the range of applications mentioned:

|          | Per cent. |
|----------|-----------|
| Carbon   | 0.3       |
| Chromium | 3.0       |
| Tungsten | 10.0      |
| Vanadium | 0.3       |

This steel exhibits a good notched bar impact-test value only on being tempered at a temperature between narrow limits, namely 620-660° C. The strength, however, falls considerably due to this tempering alone. The narrow limits for the tempering temperature are difficult to observe.

The steel according to the invention is, on the other hand, tempered to a blue colour 300° C. only, an operation which can be carried out easily and reliably in the workshop. From the following comparison it is clear that the new steel is, in respect of strength and tenacity, superior to the above given chromium-tungsten steel.

| Type of steel            | Hardened at—      | Tempered at—       | Elastic limit kg/mm <sup>2</sup> | Tensile strength kg/mm <sup>2</sup> | Elongation % | Contraction % | Notched bar impact test mkg/cm <sup>2</sup> | 60 |
|--------------------------|-------------------|--------------------|----------------------------------|-------------------------------------|--------------|---------------|---------------------------------------------|----|
| Chromium-tungsten steel. | 1,200° C. in oil. | 660° C.            | 128.0                            | 140.8                               | 7.5          | 54.8          | 7.2                                         | 65 |
| New steel.               | 11                | 330° C blue colour | 146.3                            | 167.5                               | 8.5          | 42.6          | 9.2                                         |    |

The values for elongation are those for standard test bars with a gage length of 70

11.3 √cross-section.

The notched bar impact-tenacity (work of fracture) is determined on bars of cross section 20 x 160 mm, with a 4 mm. wide, 5 mm. deep semicircular notch, the distance of the supports being 120 mm., by means of 75 mkg. Charpy-pendulum impact apparatus.

Alloying metals having an improving effect, other than chromium, tungsten and nickel, such as vanadium, may, according to the invention, be added to the steel. Further, the tungsten may be wholly or partially replaced by molybdenum, which has the same effect, and the nickel by cobalt.

What I claim is:

1. A special steel comprising 10% tungsten, 3% chromium and 3% nickel.
2. A special steel comprising 10% tungsten, 3% chromium, 3% nickel and 3% carbon.

In testimony whereof I affix my signature.

OTTO PATTERMANN.